

## UNITED STATES PATENT OFFICE

EDWARD S. MEAD, OF PHILADELPHIA, PENNSYLVANIA, ASSIGNOR OF ONE-HALF TO  
JONATHAN P. EDWARDS, OF PHILADELPHIA, PENNSYLVANIA

## DISTILLATION OF COAL

No Drawing.

Application filed August 12, 1929. Serial No. 385,467.

My invention relates to the distillation of coal, and more particularly to a process for the utilization of coal which is too fine or otherwise unsuited for commercial use, and to the novel products resulting from my process.

Specifically, I have devised a process for the commercial utilization of anthracite fines, which are a waste product, so that certain novel products which result may be successfully used commercially with large economies where ordinary high grade coal is used.

The process may be carried out on carbonaceous materials having the properties of anthracite fine coal, also known as anthracite silt, and broadly comprehends the steps of treatment of the properly prepared fines with crude oil and water whereby the combustible matter of the coal unites with the oil to produce an amalgam or plastic mass and the incombustible matter such as sand, rock dust, and slate, pass off into the water through screens, and (B) treatment of the plastic mass of combustible matter by a distillation process which distillation is arrested at a point or points whereby an entity is obtained that possesses characteristics of (1) high calorific value, (2) low ash content, and (3) a volatile content not appreciably different from high grade semi-bituminous coal.

The entity referred to as a result of step (B) herein described, has physical characteristics which permit its use as (A) a fuel per se, for heating steam boilers, or for metallurgical operations where powdered anthracite is now used, or use as a carbonizing agent in metallurgical processes; as (b) a supplementary ingredient to be mixed with soft coal and the resulting mixture used as a substitute for soft coal with certain economical advantages; as (c) an intermediate product for the making of briquets, which latter are subjected to a distillation process which is continued to complete carbonization with the final production of a smokeless and odorless fuel. Alternatively, the briquet distillation may be arrested to form various grades of fuels approaching those completely carbonized.

The process in detail is indicated by the

following example: Anthracite fines, which are now a waste product, are pulverized in a Harding or Fuller mill until 60%-80% will pass through a 200 mesh screen. The resulting product is then mixed with oil and water, about one barrel of crude oil to a ton of coal, and the mixture is then agitated in a large tank. The combustible elements in the coal unite with the oil and the incombustible matter passes off into the water through screens as it flows through the tank. This preliminary treatment is already known. The resulting amalgam of coal and oil is transferred to a retort for distillation without briquetting. The distillation of the light oils from the amalgam is conducted at a temperature below 750° Fahrenheit, preferably about 600°, and is arrested at a point which produces a product a representative analysis of which is as follows:

|                 | Per cent    |
|-----------------|-------------|
| Volatile matter | 14 to 18.03 |
| Fixed carbon    | 80 to 74.42 |
| Ash             | 7.9 to 7.55 |

The distillation process in a 100 ton per hour retort could be completed in one hour.

This product is of a fine, flour-like, gummy consistency which has a calorific value of approximately 13,500 B. t. u. As indicated hereinbefore, this product can be mixed with soft coal and the mixture burned without any loss and with great resulting economies to the user. A mixture of equal parts of my processed anthracite and bituminous coal results in considerable savings over straight soft coal. My processed anthracite coal can also be burned in powdered form without a mixture of soft coal, but in this form, the process of distillation must be carried on at higher temperatures, up to 650° Fahrenheit, so that the product may be "dry" enough to be readily handled in blowers. When an equal part of soft coal is mixed with the anthracite, the distillation can be carried out at a lower temperature, 550°, and a larger amount of oil can be left in the coal. When used in cement burning, where a short flame is required, I have found it desirable to grind the anthracite fines and soft coal together in order to obtain a uniform mixture and then

process the mixture in the manner above described. This method has the additional advantage that, in the process of distillation, especially when the soft coal in the mixture is rich in hydro-carbons, a certain amount of gas is produced from this soft coal which adds to the amount of oil recovered by the distillation.

My experiments with this product have indicated that it forms a valuable base for the manufacture of briquets, either with or without mixture with raw plastic coal amalgam from which it is produced. The briquets are distilled in the usual retort with the ultimate production of smokeless and odorless fuel and a recovery of all volatiles in the usual fractionating equipment. The briquetting of my processed anthracite eliminates difficulties of subsequent carbonization together with uneconomical considerations which pertain to the briquetting of non-distilled raw amalgam. In carbonizing briquets made from the raw amalgam, mixture of coal and oil, great difficulty is experienced in securing complete carbonization and complete recovery of the oil, for the reason, that in the carbonization process, a crust is formed on the briquets which interferes with the expulsion of the gasses from the interior of the briquets. This difficulty is obviated by carrying on the primary distillation with the material in powdered form, then briquetting the remaining material and completing the carbonization of the briquets with or without the recovery of the remaining oil which is of small amount. This method has the further advantage that a large processing plant could be located near the source of supply, and the raw material for briquetting shipped to briquetting plants, located at points of consumption. The cost of such briquetting plants would be small since they would be free from the high cost of oil recovery apparatus.

It is apparent that my process is not limited to anthracite fines. For example, it may be applied to unburned coal recovered from screened ashes at the power plant. These ashes can be pulverized, treated with oil, and processed as above indicated, to recover the unburned coal, the arrested distillation product being then mixed with soft coal and burned in power plants, or it could be briquetted. It is clear that any carbonaceous material which is amenable to treatment by step A herein described, may be processed as I have indicated. The numerical values given herein for my novel products are to be considered exemplary, rather than values of limitation.

Within the scope and spirit of my invention, I desire only to be limited by the appended claims.

I claim:

1. The process of making a solid fuel which

comprises mixing powdered anthracite coal with sufficient crude oil to form a slightly plastic mixture and destructively distilling the same at temperatures below a maximum of 750° F. for approximately one hour so as to produce a product containing from 14% to 18% volatile matter.

2. The process of making a solid fuel which comprises mixing powdered mineral, combustible, carbonizable material with sufficient crude oil to form a slightly plastic mixture and destructively distilling the same up to a temperature of approximately 600° F. for a period of time sufficient to produce a product containing from 14% to 18% of volatile matter.

In testimony whereon, I have hereunto subscribed my name this tenth day of August, 1929.

EDWARD S. MEAD.